

W. R. SEIGLE.

COMPOSITE FIREPROOF BUILDING FABRIC AND METHOD OF MAKING THE SAME.  
APPLICATION FILED APR. 8, 1919.

1,436,914.

Patented Nov. 28, 1922.

Fig. 1



Fig. 2



Fig. 4



Fig. 3



Inventor:

William R. Seigle  
by James Robert Cushman  
his Atty.

Patented Nov. 28, 1922.

1,436,914

# UNITED STATES PATENT OFFICE.

WILLIAM R. SEIGLE, OF NEW YORK, N. Y.

## COMPOSITE FIREPROOF BUILDING FABRIC AND METHOD OF MAKING THE SAME.

Application filed April 8, 1919. Serial No. 288,562.

To all whom it may concern:

Be it known that I, WILLIAM R. SEIGLE, a citizen of the United States of America, and resident of New York, in the county of 5 New York and State of New York, have invented new and useful Improvements in Composite Fireproof Building Fabrics and Methods of Making the Same, of which the following is a specification.

10 This invention relates to composite fireproof building or roofing fabrics having a cloth, paper or felt base, and a permanent protective coating of pleasing appearance for the exposed face of the fabric.

15 I am aware of many efforts in the prior art to provide a ready-fabricated roofing which can be applied with good joints so as to become practically an integral and unbroken covering for a roof; of structures 20 for such fabrics intended to make such roofings fireproof; and of fabrics for these general purposes varying in the nature and relation to each other of the component parts of the fabric or sheet for roofing. I am

25 aware, for instance, of the use of certain coating materials, such as sand or broken slate, to prevent a waterproof cementitious coating from sticking the sheets together when they are stacked or rolled, and of various attempts in the prior art to improve the 30 appearance of such coatings, or to improve the heat-resisting qualities of the material coated.

But so far as I am aware none of the prior 35 art fabrics when at all successful from the point of view of applicability to the situations in which such roofs are most desired, of cheapness, or of fireproof quality, are also successful from the points of view of 40 providing a fabric having a surface resistant to detachment under erection or long use, or when subjected to high temperature, or providing a surface agreeable to the eye.

As an element of architectural effect, such 45 sheet roofings are detrimental to the artistic appearance of surfaces covered by them, and by custom connotative of makeshift, temporary or cheap building, as well as intrinsically disagreeable either in color or in 50 surface, or in both. Heretofore when they have been really fireproof, such fabrics have also been more expensive than plastic composite roofs or walls applied in place. I am not aware of any ready-fabricated roofing 55 which presents a rough, broken or variegated

surface, nor of any in which the surfacing material is adherent to a degree rendering the coating reliably permanent.

The prime object of the present invention is to provide a composite building material 60 which can be made up in rolls or stacked in sheets for transportation and sale, such material being characterized by an improved resistance to fire, by a marked improvement in permanent adhesion of the surface coating, and by a surface having an agreeable architectural appearance both as regards texture and as regards color. Further objects are to employ in making the new fabric materials heretofore regarded as waste 65 materials, to provide a roofing material comprising a felt, paper or cloth element and a surface armoring or fireproofing element each extracted from the same natural mineral origin and balancing each other econ- 70 nomically by utilization of different parts of the same raw material, and to provide an art of making such composite fabrics. 75

In the accompanying drawings:

Figure 1 is a displayed view showing the 80 various layers of a preferred form of the fabric;

Figure 2 is a transverse section through a sheet;

Figure 3 is a greatly enlarged section 85 through the fabric; and

Figure 4 is a diagram of apparatus illustrating steps taken in one method of making the fabric.

In making the fabric, sheets of asbestos 90 fabric are coated with a cementitious adhesive rubbery compound, comprising for instance asphalt and any suitable filler, such as sand, calcined or uncalcined powdered stone, lime, ground calcareous matter or the like; and while this coating is in a hot and soft state, an armoring surface is formed upon and in relation to it by causing the adhesion to it and partial mingling with it of 95 the components of the armoring surface. 100

Referring to the drawing, a preferred form comprises at least two plies 1 and 2 of asbestos paper, felt, or cloth, or of a paper, felt or cloth predominantly composed of fibrous asbestos, fastened together in any 105 satisfactory manner. For complete waterproofing, it is preferred to saturate the asbestos plies with melted asphalt or an asphaltic compound, and to cement the plies together by a layer 3 of either the melted 110

asphalt or of an asphaltic cement of any desired composition; for instance, any one of the cements hitherto employed for cementing together similar laminae of other 5 laminated waterproof fabrics. The laminated sheet 1, 2, 3, provides a fireproof heat-insulating base of any desired thickness.

If desired, the longitudinal edges of the laminated base fabric may be strengthened 10 against stretching or tearing by incorporating between the plies one or more longitudinal strips 4 of strong paper, such as Kraft paper, some of the cement 3 being applied on both sides of the strip 4.

15 The surface of the ply 2 is now coated with a relatively thick layer 5 of sticky material. Preferably this cementitious material is the adhesive rubbery asphalt compound mentioned above, and in that case 20 the coating is applied hot, in which condition it is viscous, but plastic, flowing freely under pressure and adhering strongly to the ply 2. Upon and into the plastic and adhesive surface of the cementitious layer 25 5 the surface coating or armoring 6 is now laid. This comprises a random mixture of crushed stone and short asbestos fibre. The preferred material is crushed waste 30 serpentine rock from the asbestos mine (from which the longer fibred asbestos has been separated for making the fabric of the plies 1 and 2 and other uses) and which heretofore has accumulated as waste material. This material is crushed to such 35 fineness as will pass a  $\frac{1}{8}$  to  $\frac{1}{4}$  inch mesh screen, as desired, and comprises irregular granules of all lesser sizes predominantly gray in color, but containing frequent white, pale green, yellow-gray and nearly black 40 fragments, as well as a large proportion by volume of short, more or less separated fibres or crystals of asbestos proper, which the crushing and screening operations cause to be thoroughly commingled with the rock 45 fragments and somewhat separated from each other.

This broken and screened material is sprinkled upon the plastic hot coating 5 in a thick layer, and preferably rolled into the 50 layer 5 and the upper ply 2 of the base fabric under pressure.

The result is illustrated in Figs. 1 and 3. The larger fragments of rock 10 and 11 for instance, are driven into the coating 5, and may be pressed into the substance of layer 2, as shown, but do not penetrate, in the sense of breaking through, either the cementitious coating or the fibrous base. A film of the material 5 still separates the 55 fabric 2 and the fragment driven into it. The discrete masses of fibre in the coating are caused to penetrate to contact and binding relation with the fabric layer 2.

The plastic flow of the excess of the material 5 is effective to enter all of the in-

teriorities of the lower part of the layer 6, under these circumstances, and to adhere to the bundles 12 of asbestos fibre found everywhere in the layer 6. The result of this is to bind to the ply 2 a relatively thick conglomerate of fragments 10, 11, bundles of fibre 12, and the cementitious matter 5. A further result is to leave unbound in this conglomerate an irregular and variable portion of the layer 7 originally deposited on the fabric.

The cementitious layer 5 having sufficient 80 cooled the unbound material is now removed from the surface of the completed fabric by gravity, shaking, an air-blast, or other desired means, and may be collected for further use. The thickness of the retained coat depends upon the amount of cementitious matter in layer 5.

The completed fabric has a very rough 85 surface comprised of the irregular rock fragments firmly bound on the base, which vary among themselves greatly in color; it shows irregular pale gray or white asbestos fibre patches, a considerable number of free-ended fibres of asbestos projecting from the surface, and at the depths of recesses between the armoring fragments, it shows throughout a dark background of the asphaltic cement 5. The fibrous appearance 90 of the asbestos elements of the surface predominates, and aids in giving a surface texture very closely imitating the surface of an old weathered wooden shingle. The whole color effect of the surface is a soft 95 gray comprised of the mixed color elements of which it is composed.

A relatively large proportion of the thickness of the fabric is comprised of the 100 layer 5, 6, which as shown in Fig. 2 may be as thick or thicker than the base fabric.

The fabric may be made in other ways. For instance, I may coat the upper face 105 of base 1, 2, with a plastic cement so fluid when hot, and at such a temperature as to permit the broken rock and fibre coating to be sufficiently engaged with it by gravity, by deposit upon it by sprinkling only, without pressure, and in that case the rough surface desired will result from the different 110 sizes of the attached particles. In either mode of attaching the surface coat, the amount of coating material may be calculated by the known binding power of the cementitious layer, so that deposit of excess 115 material is avoided, but I prefer to deposit a large excess of the material in order to be able to employ pressure transmitted by the unbound excess of this material to attach the adherent portion, and in this way 120 to avoid the flatness of surface otherwise obtained by rolling the armoring coat into the plastic adhesive by a plain cylindric 125 roller, or the artificial appearance of a surface due to a roller having an artificial 130

roughened surface; and also to avoid any contact of the pressure roll with the surface-binding adhesive 5.

Under test by application of a blast 5 of flame, the coating 6 is found to be thoroughly retained, although the cement 5 was first melted and then carbonized. This is not the case with any other armoring material of which I am aware, such other coatings 10 showing a disposition to flow off when their cementitious binder softens under heat. I attribute this improved resistance to fire to the nature of the coating 6 and the mechanical adherence of its fibrous and fragmentary elements to the fabric 2 secured by the method of assembling them as described.

While the method of making the new fabric is independent of any particular apparatus and may conveniently be carried 20 out by hand, I have shown for aid in practicing it in Fig. 4 a typical set of apparatus adapted for preparing a relatively continuous web of the material. The plies 1 and 2 are impregnated and stuck together at A, 25 the ply 2 is coated with the hot cementitious layer 5 at B, sprinkled with armoring material at the shaker-screen C, an excess of material being deposited; is then, after a run of suitable length to allow the layer 5 30 to set somewhat, rolled at D, and then after a run long enough to allow further cooling of layer 5, is inverted at E, and if desired subjected to an air blast at e and shaking at e' to remove the excess of armoring material, and rolled up in a finished state at F.

What I claim is:

1. Composite fabric comprising an asbestos fabric base, an adhesive cementitious coating on said base, and an armoring coat imbedded in and held by the cementitious coating comprising fragments of stone and asbestos fibre, components of the coating projecting at irregular distances from the general surface of the coating, whereby to form 45 an irregular, rough surface.

2. Composite fabric imitating in appearance a weathered wooden shingle comprising a base-fabric, a cementitious coating thereon, and irregular particles of broken 50 stone of various colors intermingled with short fibred asbestos commingled with and covering the surface of said cementitious coating.

3. A fireproof fabric comprising a base-fabric predominantly of asbestos fibre, a 55 cementitious coating, and a fireproof armoring coating imbedded in and held in place by the cementitious coating, said armoring coating comprising a fibrous material and a comminuted mineral substance in intermixed relation.

4. A composite fabric sheet comprising laminæ of asbestos fabric fastened together by an asphaltic cement, and an armoring

coating comprising a mixture of stone fragments and discrete short-fibred asbestos held on one surface of the laminated sheet by a cementitious substance.

5. A composite fabric sheet comprising laminæ of asbestos fabric fastened together 70 by an asphaltic cement, and an armoring coating comprising a mixture of stone fragments and discrete short-fibred asbestos held on one surface of the laminated sheet by an asphaltic cement.

6. A composite building fabric comprising a base fabric consisting predominantly of fibrous asbestos, a cementitious adhesive substance for holding the different parts of the fabric in assembled relation and a rough 80 armoring coating on one face of the fabric consisting of crushed and screened serpentine rock containing discrete particles of short-fibred asbestos.

7. The art of making composite building 85 fabrics comprising coating a base fabric with a plastic cementitious substance, depositing thereon a thick layer of armoring material, forcing into said cementitious coating while it is in a plastic condition a part 90 of this layer, and then removing the unbound excess of armoring material.

8. The art of making composite building fabrics comprising coating a base fabric with a plastic cementitious substance, applying 95 to said cementitious coating while it is in a plastic condition a mass of discrete fragments of rock and a fibrous material, and placing the applied mass under pressure to commingle some of it with the cementitious 100 coating.

9. The art of making composite building fabrics comprising coating a base fabric with a plastic cementitious substance, applying to said cementitious coating while it is 105 in a plastic condition a mass of discrete fragments of rock and a fibrous material, placing the applied mass under pressure to commingle some of it with the cementitious coating, and thereafter removing the excess 110 of the fragments of rock and fibrous material not engaged and bound by the plastic flow of the cementitious substance.

10. The art of making composite building fabrics comprising coating a base fabric 115 with an asphaltic cementitious substance in a hot and plastic state, applying to said cementitious coating while in such state an armoring coating of mixed fragmentary stone and fibrous material in excess of an 120 amount adapted to be bound by adhesion to the cementitious coating, causing adhesion by pressure on the excessive amount of armoring coat and then removing the unbound excess of the armoring material.

Signed by me at New York, N. Y., this 125  
4th day of April 1919.

WILLIAM R. SEIGLE.